

No. 812,493.

PATENTED FEB. 13, 1906.

W. HOSKINS.

METHOD OF GRANULATING ALUMINUM.

APPLICATION FILED AUG. 26, 1904.



Witnesses:

W. C. Wright.

Walter N. Winberg.



Inventor:

William Hoskins,

Bridgnorth, Shropshire, Eng.

Attest:

# UNITED STATES PATENT OFFICE.

WILLIAM HOSKINS, OF LAGRANGE, ILLINOIS.

## METHOD OF GRANULATING ALUMINIUM.

No. 812,493.

Specification of Letters Patent.

Patented Feb. 13, 1906.

Application filed August 26, 1904. Serial No. 222,210.

*To all whom it may concern:*

Be it known that I, WILLIAM HOSKINS, a citizen of the United States, residing at La-  
5 grange, in the county of Cook and State of Illinois, have invented a new and useful  
Method of Granulating Aluminium, of which  
the following is a specification.

My invention relates to an improved  
method of treating aluminium for the purpose  
10 of reducing it to a more or less finely-divided  
condition.

The various methods hitherto employed  
for granulating aluminium are all of them, so  
far as I am aware, quite slow and laborious,  
15 and as there is a large and increasing demand  
for granulated aluminium the question of the  
cost of its production has become one of ma-  
terial importance.

My object is to provide a method in the  
20 practice of which aluminium may be quickly  
and easily reduced to any desired degree of  
fineness, thus materially lessening the cost of  
the product.

My improved method consists in melting a  
25 mass of the metal, then stirring the molten  
mass in the presence of an oxidizing agent  
and continuing the stirring uninterruptedly  
or otherwise until the mass cools and solidifies.  
The mass may be melted in a crucible,  
30 and the agitation may be produced by stir-  
ring the mass in the same crucible in a man-  
ner to expose the mass throughout to the ox-  
idizing effect of atmospheric air. As the mass  
becomes cool and plastic more or less finely-  
35 divided portions thereof, which have been  
subjected to physical contact with the air, be-  
come superficially coated with extremely  
thin oxid films possessing a higher melting-  
point than the metal. The oxid films act as  
40 envelopes for the particles of metal and have  
a tendency to keep the particles formed by  
the agitation from reuniting. Thus the alu-  
minium may be very quickly and cheaply re-  
duced to any state of division—from impalpa-  
45 ble powder to coarse particles—depending  
upon the degree of agitation and the length  
of time employed in carrying on the method.

In the accompanying drawings I show ap-  
paratus capable of use in carrying out my  
50 method in a small way.

Figure 1 is a vertical section, and Fig. 2 a  
section on line 2 in Fig. 1.

A is a crucible, and B a frame or stand in  
which the crucible may be removably clamped  
55 by means of the set-screw a. Journaled in the

frame is a vertical pipe C, to which is fastened  
a pair of companion-plates b, carrying stirrer-  
rods c. Also fastened to the pipe C is a gear-  
wheel d, rotated from a pinion e on the shaft  
f, having an operating crank or handle g. 60

In practice the aluminium to be treated by  
my method is melted in the crucible A, after  
which the crucible is placed in the frame B to  
occupy the position shown, wherein the pipe  
and stirrer rods extend downward in the 65  
molten mass nearly to the bottom of the cru-  
cible. Turning the handle g causes the pipe  
to rotate and the rods c to swing around and  
stir the mass. The effect of this stirring is to  
70 agitate the molten aluminium and cause sub-  
stantially all parts of the mass in a short time  
to be carried into physical contact with the  
atmosphere at the top of the crucible and be-  
come oxidized. The crucible contents thus  
75 soon become a mass of molten particles en-  
veloped in extremely thin oxid films, and as  
these oxid films remain infusible they tend to  
keep the particles from running together or  
reuniting. The longer or more rapidly the  
80 stirring operation is performed before the par-  
ticles cool to solidity the finer the state of di-  
vision of the mass. Thus the operator may  
with reasonable accuracy readily effect the  
result in this regard that he wishes to obtain.  
To quicken the operation and to aid the 85  
same when it is desired to produce a very fine  
state of division of the metal, air or other ox-  
idizing-gas may be forced into the mass. At  
the top of the pipe C is a swivel-coupling h, to  
90 which a hose or the like may be attached.  
The hose would connect with a pump or other  
device for supplying air or other oxidizing-  
gas under the necessary pressure. The gas  
thus forced into the lower part of the recepta-  
95 cle would of itself tend to agitate and impreg-  
nate the mass; but I prefer to employ there-  
with the stirring means described.

The means described may be variously  
modified without departing from the spirit of  
my invention as set forth in the appended 100  
claims.

What I claim as new, and desire to secure  
by Letters Patent, is—

1. The method of reducing aluminium, and  
other metals the oxids of which have a high 105  
melting-point, to a more or less finely-divided  
condition, which consists in forcing an ox-  
idizing-gas into the molten mass to impregnate  
the same, at the same time agitating the  
mass, and continuing the agitation while the 110

mass is cooling, thereby causing the mass in solidifying to separate into superficially-oxidized particles.

2. The method of reducing aluminum, and other metals, the oxids of which have a high melting-point, to a more or less finely-divided condition, which consists in forcing an oxidizing-gas into the molten mass, at the same

time mechanically stirring the mass, and continuing the stirring while the mass is cooling, thereby causing the mass in solidifying to separate into superficially-oxidized particles.

WILLIAM HOSKINS.

In presence of—

WALTER N. WINBERG,  
L. HEISLAR.